

## UNITED STATES PATENT OFFICE

2,357,653

## METHOD OF CASTING

Herbert M. E. Heinicke, Elgin, Ill., assignor to  
 Western Electric Company, Incorporated, New  
 York, N. Y., a corporation of New York

No Drawing. Application December 10, 1941,  
 Serial No. 422,329

4 Claims. (Cl. 75—160)

This invention relates to a method of casting and more particularly to a method of casting a copper silicon manganese alloy.

In the casting of certain alloys, wherein silicon or manganese are employed, it has been regarded as necessary to postpone the addition of the silicon or manganese until just prior to the pouring, the belief being that the silicon or manganese would be burned off if added earlier. Adding these ingredients just prior to pouring has, however, caused "boiling" in the mold and resulted in the formation of air pockets in the castings which render them unfit for certain uses.

An object of the present invention is to provide an effective and efficient method of reducing porosity in castings.

One embodiment of the invention contemplates adding metallic silicon and copper manganese to a melt of copper approximately one hour prior to the pouring thereof.

Other objects and advantages will be apparent from the following detailed description of an embodiment thereof.

In practicing this invention, a charge of approximately 1170 pounds of copper is placed in a standard induction furnace and brought to a temperature of 1900° Fahrenheit. At this point, 38 pounds of metallic silicon containing about 98% silicon and 42 pounds of copper manganese containing about 30% manganese are added to produce a total charge of 1250 pounds. A loss of about  $\frac{1}{10}$  of one percent metallic silicon and copper manganese occurs prior to the pouring; thus a charge of this proportion will produce a final alloy composing approximately 3% silicon, 1% manganese, and the rest copper. The churning action of the metal in the furnace causes these ingredients to be thoroughly mixed. A covering of charcoal is maintained on the charge, and sufficient salt is added to keep the slag fairly thin. The heating of the charge is continued until it reaches a temperature of from 2230 to 2250° Fahrenheit, at which time it is poured. The metallic silicon and copper manganese are added at 1900° Fahrenheit because it has been found to take approximately one hour in a standard induction furnace for the charge to be heated from 1900° to the pouring temperature of 2250° Fahrenheit.

Contrary to metallurgical theory it has been found that this process does not result in undue burning out of the silicon or manganese. As stated above, a loss of  $\frac{1}{10}$  percent has been found to occur. Such a loss may be regarded as negligible. It will be obvious that the proportions of

silicon, manganese and copper in the final alloy may be easily varied by adding more or less metallic silicon and copper manganese as may be required. In practice, the composition of the final alloy has been varied with satisfactory results as follows:

|                    | Per cent     |
|--------------------|--------------|
| Manganese          | .55 to 1.35  |
| Silicon            | 2.85 to 3.35 |
| 10 Balance copper. |              |

To produce a copper silicon manganese alloy of any particular proportion within this range, it is only necessary to add approximately  $\frac{1}{10}$  of 1% more metallic silicon and copper manganese than is desired in the final alloy.

By adding metallic silicon and copper manganese an hour prior to the pouring, the tendency of the metal to boil in the mold on pouring is totally eliminated, and the porosity of the cast alloy is substantially reduced. When employing this method, it has been found unnecessary to reject any castings although with methods previously employed, rejections were frequent.

A similar process has been successfully employed in casting manganese brass. Here again the manganese was added an hour prior to the pouring with greatly improved results and no serious loss of manganese.

It will be understood that the nature and embodiments of the invention herein described are merely illustrative and many changes and modifications may be made therein without departing from the spirit and scope of the invention.

What is claimed is:

1. A process of making a copper alloy containing from .55% to 1.35% of manganese and 2.85% to 3.35% silicon which comprises heating the copper to a temperature of about 1900° F., adding the silicon and manganese an hour prior to reaching pouring temperature, and raising the metal to the pouring temperature.

2. A process of making a copper alloy containing from .55% to 1.35% of manganese and 2.85% to 3.35% silicon which comprises heating the copper to a temperature of about 1900° F., churning the molten metal as by heating in an induction furnace, adding the silicon and manganese, heating the metal to a temperature of about 2250° F. over a period of time sufficient to cause said silicon and manganese to alloy with the copper, and then casting the metal.

3. A process of making a copper alloy containing from .55% to 1.35% of manganese and 2.85% to 3.35% silicon, which comprises heating the

copper to a temperature of about 350° F. under the pouring temperature, adding the silicon and manganese at said temperature, raising the metal to the pouring temperature, and then casting the metal.

4. A process of making a copper alloy containing from .55% to 1.35% of manganese and 2.85%

to 3.35% silicon, which comprises heating the copper to a temperature of about 1900° F., adding the silicon and manganese an hour prior to reaching pouring temperature, raising the metal to the pouring temperature, and then casting the metal.